

[54] **PROCESS FOR THE CONTINUOUS TREATMENT OF TEXTILE MATERIALS**

8/151.2; 68/DIG. 5, 5 D, 5 E, 9, 177; 28/1.6;  
34/115

[75] Inventor: **Heinz Fleissner**, Egelsbach, near Frankfurt, Germany

[56] **References Cited**

UNITED STATES PATENTS

|           |         |                 |          |
|-----------|---------|-----------------|----------|
| 3,126,556 | 3/1964  | Fleissner ..... | 8/151.2  |
| 3,242,702 | 3/1966  | Fleissner ..... | 68/177 X |
| 3,288,551 | 11/1966 | Raff .....      | 8/21     |

[73] Assignee: **Vepa AG**, Basel, Switzerland

[22] Filed: **Apr. 18, 1973**

[21] Appl. No.: **352,348**

**Related U.S. Application Data**

[63] Continuation of Ser. No. 13,988, Feb. 25, 1970, abandoned, Continuation-in-part of Ser. No. 831,952, June 10, 1969, abandoned.

[30] **Foreign Application Priority Data**

Feb. 26, 1969 Germany ..... 1909646  
Jan. 31, 1970 Germany ..... 2004390

[52] **U.S. Cl.** ..... **8/149.1, 8/149.3, 68/DIG. 5, 68/5 D**

[51] **Int. Cl.** ..... **B05c 9/14, D06c 1/08, D06c 7/02**

[58] **Field of Search** ..... 8/149.1, 149.3, 151, 152,

*Primary Examiner*—Harvey C. Hornsby

*Assistant Examiner*—Philip R. Coe

*Attorney, Agent, or Firm*—Craig & Antonelli

[57] **ABSTRACT**

The present disclosure is directed to a process for the continuous treatment of fibrous and thread-like materials in the form of slivers, roving or fibrous ribbon wherein uniform treatment, for example, uniform dye application and uniform setting of the dyestuff is effectively achieved.

**8 Claims, 2 Drawing Figures**



PATENTED SEP 17 1974

3,835,490

SHEET 1 OF 2



Fig. 1

Inventor:

HEINZ FLEISSNER

By Craig Antonelli, Stewart & Hell  
Attorneys

PATENTED SEP 17 1974

3,835,490

SHEET 2 OF 2

Fig. 2



Inventor:

HEINZ FLEISSNER

BY

Craig, Antonelli, Stewart & Hell  
Attorneys

**PROCESS FOR THE CONTINUOUS TREATMENT  
OF TEXTILE MATERIALS**

The present application is a continuation of application Ser. No. 13,988, filed Feb. 25, 1970, and now abandoned, which is in turn a continuation-in-part of application Ser. No. 831,952, filed June 10, 1969 and now abandoned.

**BACKGROUND OF THE INVENTION**

The present invention relates to a process for the continuous treatment, particularly dyeing, of textile materials, preferably fibrous and thread-like materials, for example, synthetic fibers, such as polyester and polyamide fibers. According to the present invention the materials to be treated is continuously conveyed through several treatment steps, such as, for example, impregnating and/or printing the textile material with dye, setting the dyestuff, utilizing a temperature treatment compatible with the fiber being treated, such as for example, steaming the material in saturated steam, or thermosoling the material at a temperature of about 170°-230°C. utilizing air, wherein the treatment medium is conducted in each case through the material by means of a suction draft. Finally, the textile material is washed and dried.

The parent application relates to an apparatus consisting of several devices wherein, due to the use of said devices and the construction thereof, it is not only suitable for the continuous treatment of woven and knitted goods, cables and combed yarns by the thermosol process, but it is also suitable for the treatment of said materials in a saturated steam atmosphere. Furthermore, it is effective for treating loose fibrous materials, such as for example, cotton flock for the purpose of continuously bleaching or dyeing said material. This apparatus and the individual devices required therefor present an effective arrangement for the efficient management and reduction in the necessary capital outlay for the treatment of textile fibers.

In addition to the above-mentioned textiles, it is also conventional to dye yarn in the form of strands or spools in a discontinuous manner. It has also been suggested to dye and/or print yarns in a continuous fashion. In this process, a plurality of yarn threads pass through the individual treatment units and are thereafter wound up again. However, in the continuous dyeing of yarns, it is difficult to apply the dyestuffs uniformly to the individual fibers and to attain a uniform setting throughout. Also some difficulties are encountered in washing the dyed, twisted yarns satisfactorily. A deficient setting (fixing) and washing process produces a lower rubbing resistance (fastness to rubbing) in the fabric.

**SUMMARY OF THE INVENTION**

An object of the present invention is to avoid the prior art disadvantages in the continuous treatment of textile materials.

Another object of the present invention is to provide an improved process for the continuous treatment of textile materials, for example, fibrous and thread-like materials in the form of silvers, roving or fibrous ribbon.

A further object of the present invention is to provide an improved process for dyeing fibrous and thread-like

materials, and to render the utilization of the apparatus suggested in the parent application even more versatile.

Other objects and further scope of applicability of the present invention will become apparent from the detailed description given thereafter; it should be understood, however, that the detailed description and specific examples, while indicating preferred embodiments of the invention are given by way of illustration only, since various changes and modifications within the spirit and scope of the invention will become apparent to those skilled in the art from this detailed description.

Pursuant to the present invention, it has been found that the above-mentioned disadvantages may be eliminated and a much improved process for the continuous treatment of textile materials may be obtained by providing that the fibrous and thread-like materials are subjected to the dyeing and/or printing treatment not in the form of a yarn, but rather in the form of a silver, or as a roving or fibrous ribbon (slubbing) in case of endless synthetic threads.

Conducting the dyeing step with untwisted material affords the advantage that it is now possible to apply the dyestuffs flawlessly and uniformly and to effect a substantially more uniform setting and washing treatment, since the respective treatment media can now flow around the individual threads on the loose fiber arrangement. Similarly, as is known in the continuous yarn dyeing method, it is also advantageous in this instance to treat a plurality of such slivers, or rovings or fibrous ribbons continuously, combining them into the shape of a fibrous web.

In order to be able to set a large amount of material in a space-saving arrangement, it is suggested to heat the sliver and the like, after the dyestuff application, to the setting temperature and then to place this material into folds (pleats) and expose it in this folded condition to at least the dyestuff setting treatment. Depending on the washing and drying elements employed, this folded condition can also be retained during the washing and drying stages of the process. Heating the sliver to the setting temperature prior to folding has the advantage that it makes a completely uniform and shock-like (sudden) heating possible. In many cases, it is advantageous to remove the folded condition after the setting treatment and prior to the washing or drying step, and to subject the slivers and the like to the additional treatments, for example washing and drying, in the form of a web. In this connection, it is important that the treatments take place without tensioning (stretching). This is readily possible when the process is conducted on so-called sieve drum washing machines and sieve drum dryers, or also on perforated belt washing machines and perforated belt dryers.

The apparatus for conducting the above-mentioned treatment according to the present invention advantageously comprises the following individual elements:

60 A draw-off device for drawing material from spools, coils, or from cans, and for combining a plurality of slivers, rovings, or fibrous ribbons into a web;

65 a dye application device, for example a padder, suitable for this purpose and/or a printing device. A typical padder which can be used is, for example, a wedge padder;

a setting unit, for example, a steaming device;

A washing device which can comprise, for example, several treatment baths, each provided with a sieve drum;

a drying unit, especially a sieve drum dryer;  
a depositing or windup device: It is advantageous, in this connection, to wind up the individual slivers in each case individually; and  
a common control device for the above-mentioned units.

It is suggested to employ, as the setting unit, a perforated belt steamer with at least one sieve drum subjected to a suction draft, said sieve drum being disposed in front of the perforated belt.

A particular advantage of the apparatus of the present invention is that it can be utilized for all of the known textile fibers for the optimum treatment thereof. Synthetic fibers, such as polyacrylic fibers or polyacrylonitrile fibers, and natural fibers such as wool, cotton, or cellulose-base fibers are treated under saturated steam conditions at about 100°-102°C. This treatment effects the setting of the dyes disposed thereon, or the bleaching of the fibers by means of bleaching agents added thereto. In order to obtain a sufficient setting of the colors, and especially for the bleaching process, a longer dwell time of the textile material in the treatment chamber is necessary. The duration of this residence time extends from about 3-20 minutes. In contrast thereto, polyester fiber is treated in accordance with conventional thermosol method, for which purposes a temperature of above about 170°C., preferably 190°-210°C. must be maintained in the treatment chamber. As the treatment medium, air or superheated steam can be employed. The residence time can be from 20 seconds up to about 1 minute. In addition to polyester fiber, polyacrylic fiber can also be treated by means of the thermosol process.

This apparatus, which is insulated with respect to the outside air, and the inlet and outlet of which are sealed against the outside atmosphere, for example, by means of a pair of inlet rolls and outlet rolls, can also provide, as seen in the conveying direction of the materials, several sieve drums disposed in series, the material being treated alternately contacting said sieve drums. On these sieve drums, the textile material is exposed to an intensive throughflow of the treatment medium, which heats up the material in a shock-like fashion. The penetration of the textile material by the treatment medium is effected on both sides of the material as it is alternately conveyed on the surface of the sieve drum means. An endless conveyer belt follows this unit, on which belt the textile material is conveyed in the folded condition through the remaining length of the device either rapidly or slowly, depending on the necessary residence time.

By means of an additional feature of the present invention, the setting unit can be improved in its construction so that it is even more economical and possesses even greater versatility in its utilization. According to the present invention, this is attained by providing that the conveyor belt extends from the outlet through the steam chamber to the inlet, but beneath the sieve drums which are arranged in series at the inlet. By means of this feature, it is possible to expose the fibrous material to the treatment medium either for a longer or shorter period of time without changing the construction of the setting device, and the rotational speeds of the sieve drums and the conveyor belt. In

case the conveyor belt extends to the inlet beneath the sieve drums, for example, beneath drums disposed in a side-by-side relationship, the textile material is either guided on the surface of only the first sieve drum, depending upon the requirements, or on the surface of all of the sieve drums. In the former situation, the fibrous material passes over only the first drum and then is transferred to the perforated belt disposed therebelow, if desired in a folded condition. In this situation, the

10 fans producing the vacuum within the subsequent sieve drums would have to be switched off. Since the perforated belt is operated at a slower conveying speed when compared to the sieve drums; the textile material thus remains in the setting unit for a longer period of time.

15 In case it is unnecessary for the textile fibers to remain in the setting unit for a longer period of time, which is particularly applicable in connection with the thermosol treatment of polyester fibers, the fibrous material is transported, alternatingly, over the surface of one 20 of the series-connected sieve drums, thus over-shooting and undershooting the drums. The textile materials is thereby deposited onto the conveyor belt by only the last drum, from the top in the downward direction. The material thus remains on the belt only for a short length 25 and for a short time.

#### BRIEF DESCRIPTION OF THE DRAWINGS

These and further features, advantages and objects of the present invention will become more apparent from 30 the following description when taken in conjunction with the accompanying drawings which show, for purposes of illustration only, and wherein

35 FIG. 1 is a sectional view of an apparatus for the treatment of sliver or roving in accordance with the present invention; and

FIG. 2 shows another embodiment of the setting device used in the system of FIG. 1.

#### DETAILED DESCRIPTION OF THE DRAWINGS

40 Referring now to the drawings and, in particular to FIG. 1, the slivers 1 are drawn off the spools 2 and fed, via a roller conveyor 3 as well as a pair of draw (feed) rolls 4, to a wedge padder (nip padder) 5. The slivers, rovings, and the like impregnated with dye liquor then pass to a conveyor belt 6 and into a steaming device 7. The steaming device consists of a sieve drum 8 subjected to a suction draft, and a conveyor belt 9. The conveyor belt 6 is fashioned as a perforated belt and is 45 extended around the sieve drum 8. The slivers 1 are heated to the setting temperature on the sieve drum 8 and then, radially buckled so that they are in a pleated condition when deposited on the perforated belt 9. A pair of draw-off rolls 10 are disposed at the end of the steaming unit 7, to take up the pleats. Thereafter, the 50 slivers and the like are washed out on sieve drum washing baths 11 provided with presses 12 disposed therebehind. A sieve drum dryer 13 containing sieve drums 14 subjected to a suction draft serves for drying the material. This sieve drum dryer 13 is provided with a chute 55 15 at the outlet thereof, said chute being fashioned as a dwell trough. From the dwell trough, the slivers 1 are fed to a windup device 16 where the individual slivers are again wound up.

60 Such units can effectively operate with 150 meters, and more. Depending on the number of slivers, these devices exhibit operating widths of up to about 1,200 mm. to 1,800 mm., or even more.

The setting device according to FIG. 2 consists of a heating section denoted by 20 and a residence (dwell) section denoted by 21. The heating section consists essentially of three series-disposed sieve drums 17 through 19 which convey the textile material 23, fed from the outside through an inlet 22 into the heat-insulated housing 7, through the heating section 20 so that the material alternately overshoots and undershoots the drums. Each of the three sieve drums 17 through 19 is conventionally associated with fans (not illustrated) which create a suction draft within the sieve drum. The treatment medium which is drawn into the sieve drum is recycled back to the outer surface of the sieve drum by way of regenerating or heating units, which are likewise not illustrated. The heating units can be disposed anywhere in the circulation zone of the treatment medium.

Once the fibrous material is sufficiently heated, it is passed from the top downwardly to the perforated belt 9 disposed underneath the sieve drums. The perforated belt 9 extends along the entire length of the device, i.e., along the heating section as well as through the residence section. Because of this feature, and with the fans of sieve drums 18 and 19 being switched off, the textile material can be deposited from the first sieve drum 17 onto the conveyor belt 9, also in pleats. The residence time on the conveyor belt 9, which has a slower conveying speed when compared to the sieve drums, is necessary, especially when conducting the steaming step under a normal atmosphere, i.e. under saturated steam when treating various synthetic and natural fibers.

In case the illustrated apparatus is to be employed for thermosoling, for example, polyester fibers, the textile material passes over all three sieve drums 17 through 19, alternately overshooting and undershooting the same. The material is then transferred to the conveyor belt 9, the speed of which can be optionally increased, only by the last sieve drum 19. Consequently, although the residence time can be considerably shorter, the advantage of subjecting the textile material intensively to the treatment medium, by the suction draft with alternating contact on the sieve drum surface, can be exploited.

The material which can be treated by the process and apparatus of the present invention include any of the natural or synthetic fibers. The natural fibers can include cotton, wool, silk, cellulose, etc., and the synthetic fibers may comprise synthetic polymers such as polyolefins, e.g., polyethylene, polypropylene, etc. polyamides, e.g., Nylon 6 obtained by the condensation of caprolactam, nylon 66 obtained by the condensation of hexamethylenediamine with adipic acid, etc., polyesters, e.g., polyethylene terephthalate, etc., phenolic resins, e.g. phenol formaldehyde resins, urea formaldehyde resins, etc., polyvinyl materials, e.g. polyvinyl chloride, polyvinyl acetate, etc., and acrylate resins, such as e.g., polymethylmethacrylate. Copolymers of these materials with one another or with ethylenically unsaturated monomers, and similar type polymers are also encompassed by the present invention. The present invention is also applicable to blends of the above-mentioned textile materials.

The invention being thus described, it will be obvious that the same may be varied in many ways. Such variations are not to be regarded as a departure from the spirit and scope of the invention, and all such modifications as would be apparent to one skilled in the art are intended to be included.

What is claimed is:

1. A process for the continuous treatment of fibrous and thread-like textile materials in the form of slivers, 10 rovings or fibrous ribbons which comprises impregnating or printing a textile material with a dyeing liquor; dye-fixing the dye-containing material in a single setting apparatus by conveying the material through a heat-insulated chamber of the apparatus on the conveying surface of at least one of a plurality of sieve drum means subjected to a suction draft in a heating section and then on a surface of a perforated conveyer belt in a dwell section, by drawing a heated gas through said textile material on said sieve drum means, and by 15 maintaining the heated gas around said textile material on said perforated belt; said textile material being dye-fixed on one sieve drum means and then on a surface of said conveyor belt when the heated gas is saturated steam and on a plurality of sieve drum means and then 20 on a surface of said conveyor belt when the heated gas is air at an elevated temperature or superheated steam, whereby the residence time of the material on said perforated belt is greater when the heated gas is saturated steam; washing the dyed material by conveying the material through a washbowl and then drying the material.
2. The process of claim 1, wherein the thread-like materials are selected from the group consisting of polyester fibers and polyamide fibers.
3. The process of claim 1 wherein the dye fixing is effected in an atmosphere of saturated steam.
4. The process of claim 1, wherein the dye fixing is effected in an atmosphere of air heated at a temperature of about 170° to 230°C.
5. The process of claim 1, wherein said at least one of the sieve drum means is rotating at a faster speed than the conveyor belt, thus depositing the material in the form of pleats on the surface of the conveyor belt, the material being subjected to dye-fixing in said pleated condition.
6. The process of claim 5, wherein the pleats are removed prior to washing and drying the textile material and the material is exposed to the subsequent washing and drying stages in the shape of a web.
7. The process of claim 1, wherein said textile material is natural and synthetic fibers selected from the group consisting of polyacrylic fibers, polyacrylonitrile fibers, wool, cotton and cellulose-base fibers, said textile material being treated with saturated steam at a temperature of about 100° to 102°C. for a period of about 2 to 20 minutes in said heat-insulated chamber.
8. The process of claim 1, wherein said textile material is polyester and polyacrylic fibers, said textile material being treated with air at a temperature of about 190° to 210°C. for a period of about 20 seconds to 1 minute in said heat-insulated chamber.

\* \* \* \* \*